

Patented Nov. 6, 1928.

1,690,426

# UNITED STATES PATENT OFFICE.

NORMAN E. OLIVER, OF NEW YORK, N. Y., ASSIGNOR TO HERMETITE CORPORATION, OF NEW YORK, N. Y., A CORPORATION OF NEW JERSEY.

## PROCESS FOR THE COATING OF PERVERSUS MATERIAL.

No Drawing.

Application filed May 29, 1925. Serial No. 33,635.

My invention relates to processes for the treatment of fabrics and other pervious materials and refers particularly to the treatment of such materials with the retention of softness and pliability.

It is frequently desirable to cover, or coat, pervious materials, as for instance woven fabrics, with a surface material for purposes of rendering them water proof or fire proof or

for decorative or other purposes.

The coating materials employed for this purpose may be lacquers, varnishes, cellulose or celluloid compounds and mixtures which impart valuable properties to the materials thus treated.

The employment of these, and similar, coating materials has been considerably limited because of the harshness of the treated results. Attempts have been made to overcome this objectionable quality by incorporating softening materials with the coating compounds or employing them in the coating process.

Among the softening agents thus employed are vegetable oils, such as castor oil, their sulphonated products and other oils and greases. Many of these oils are objectionable because of their rancidity, liability to injure the fiber and tendency to break down the coating compound with the formation of objectionable products.

I have found that there are two general reasons for the reduction of the pliability of materials of the character described when they are coated, or covered, with the mentioned and similar coating compounds.

The one reason is the stiffness and non-pliability of the coating compound itself, which permeates the fabric, whether the material be passed through a solution of the coating compound or the solution be applied to the ordinary woven or pervious material. This positioning of the coating compound within the fabric and between and around the fibers results in material having the physical properties of the coating compound to a large degree. This decreased pliability of the fabric is still further enhanced by the fact that the coating compounds are usually of such a nature as to adhere to the fibers, thus producing a practically solid mass of the coating compound with the fibers enclosed therein.

The other general reason for the production of coated goods of less pliability than

the original material is based upon the fact that in many coating operations, and especially in those methods in which the fabric is immersed in a solution of the coating compound, a proportion of the contained fiber oils, fats and softening agents is removed and in these cases the original pliability can not be regained by attempted replacement of the removed products.

It is evident, therefore, that the logical method for coating fabrics and other pervious materials is the retention of the original oils, the non-saturation of the material with the coating compound and the employment of a pliable coating compound.

The process of my invention possesses all of the last described desirable attributes, overcomes all of the objectionable features incident to previously known methods, and produces a coated material possessing softness and pliability.

All pervious materials have a plurality of openings therethrough, those in woven fabrics being the spaces between the several fibers. These openings have capillary attraction, the degree of capillarity being dependent upon the size of the openings, and it is through the medium of this capillary attraction that the solution of coating compounds is drawn, or carried, into the interior of the fabric. I overcome this objectionable feature by mechanically reducing the size and number of these openings.

This mechanical treatment has two effects upon the material. It reduces the size and number of the material openings and also produces a much smoother surface to the material, so that the coating compound forms a layer upon the outer face of the material, and practically prevents the formation of imbedded immovable fibers within the coating compound.

In order to retain the original softening materials within the pervious material, I coat the material upon one side only and I employ a coating compound which has high pliability.

The following is one example of the process of my invention:—

I pass the woven fabric through a high pressure friction calender which flattens the loose fibers and reduces the size of the openings. I then treat one side of the fabric with a pliable coating material, as a solution containing 100 parts of nitrocellulose to over 110

60 parts of tricresylphosphate, and dry. During the coating treatment, the coating material does not penetrate the fabric because the pores, or openings, therein have been 5 largely closed by the mechanical pressure treatment. If I am desirous of still further increasing the pliability and appearance, I can treat the fabric with a satisfactory softening agent, which can be readily and economically applied to the uncoated face of the fabric, or I can apply steam or moisture thereto which will swell the individual elements, or fibers, of the material, reproducing the natural appearance of the material 10 upon the coated side. For purposes of convenience I refer to these treatments as "after-treatments".

Any adapted softening agent can be employed, such as are well known in adaptability for such use; for instance, water-soluble oils or soap, odorless emulsified castor oil, olive oil, cotton-seed oil, or the like, the softening agent being used in its application 20 to the fabric as a thin solution.

25 It will thus be seen that by my process, I can economically produce coated pervious materials possessing great pliability without danger of injuring the material-composing ingredients or elements.

30 By "coating compounds" and "coating materials" in my specification and claims, I mean those products, either singly or in combination, which can be applied to pervious materials and which become affixed thereto by the 35 steps of my process.

I do not limit myself to the particular materials, quantities, temperatures or steps of process particularly described, as these are given in order to clearly explain the process 40 of my invention.

What I claim is:—

1. In a process for coating a pervious material, first subjecting said material to mechanical treatment whereby the openings or 45 interstices therein are reduced in size and the fibres are flattened to enhance smoothness of the surface, then applying to the surface of the material a coating compound of the class comprising cellulose, celluloid compounds or mixtures, lacquers, varnishes or the like, and having a high degree of pliability 50 when dried and forming upon the outer face of the treated material only one layer which does not permeate and embed the fibres, whereby the formation of embedded immovable fibres 55 within the layer coating is precluded, and then drying said single-layer surface coating to produce the completely finished product.

60 2. In a process for coating a pervious material, first subjecting said material to mechanical treatment whereby the openings or interstices therein are reduced in size and the fibres are flattened to enhance smoothness 65 of the surface, then applying to the surface

of only one side of said material a coating compound of the class comprising cellulose, celluloid compounds or mixtures, lacquers, varnishes or the like, and having a high degree of pliability when dried and forming 70 upon the outer face of the treated material only one layer which does not permeate and embed the fibres, whereby the formation of embedded immovable fibres within the layer coating is precluded, and then drying said 75 single-layer surface-coated side to produce the completely finished product.

3. In a process for coating a pervious material, first applying pressure to said material whereby the openings or interstices 80 therein are reduced in size, then applying to the surface of only one side of said pressed material a coating compound of the class comprising cellulose, celluloid compounds or mixtures, lacquers, varnishes or the like, and 85 having a high degree of pliability when dried and forming upon the outer face of the treated material only one layer which does not permeate and embed the fibres, whereby the formation of embedded immovable fibres 90 within the layer coating is precluded, and then drying said single-layer surface-coated side to produce the completely finished product.

4. In a process for coating a pervious material, first subjecting said material to mechanical treatment whereby the openings or interstices therein are reduced in size and the fibres are flattened to enhance smoothness 100 of the surface, then applying to the surface of one side of said material a solution containing approximately 100 parts of nitrocellulose to over 60 parts of tricresylphosphate and forming a pliable layer coating which does not permeate and embed the fibres, and 105 then drying said coating to produce the finished product.

5. In a process for coating a pervious material, first applying pressure to said material whereby the openings or interstices therein are 110 reduced in size, then applying to the surface of one side of said pressed material a solution containing approximately 100 parts of nitrocellulose to over 60 parts of tricresylphosphate and forming a pliable layer coating which does not permeate and embed the fibres, and 115 then drying said coating to produce the finished product.

6. In a process for coating a pervious material, mechanically reducing the size of the openings in said material, treating one side of said material with a coating material of the class comprising cellulose, celluloid compounds or mixtures, lacquers, varnishes or the like, and which will remain pliable in the 120 coating, drying said coating, after-treating the material, and again drying.

7. In a process for coating a pervious material, applying pressure to said material whereby the openings or interstices therein 125

are reduced in size, treating one side of said material with a coating material of the class comprising cellulose, celluloid compounds or mixtures, lacquers, varnishes or the like, and which will remain pliable in the coating, drying said coating, after-treating the material, and again drying.

8. In a process for coating a pervious material, mechanically reducing the size of the openings in said material, treating one side of said material with a solution containing 100 parts of nitrocellulose to over 60 parts of tricresylphosphate, drying said solution, after-treating the material, and again drying.

15 9. In a process for coating a pervious material, first subjecting said material to mechanical treatment whereby the openings or interstices therein are reduced in size, applying to one face of said treated material a

20 coating material of the class comprising cellulose, celluloid compounds or mixtures, lacquers, varnishes or the like, and which will remain pliable in the coating, drying said coating and then after-treating the uncoated 25 face of the material with an agent whereby the pliability and natural appearance of the treated and coated material is enhanced.

10. In a process for coating a pervious material, first applying pressure to said material whereby the openings or interstices therein are reduced in size, then applying to one side of said pressed material a coating 30 material of the class comprising cellulose, celluloid compounds or mixtures, lacquers, varnishes or the like, and which will remain 35

pliable in the coating, drying said coating, and then after-treating the uncoated face of the pressed material with an agent whereby the pliability and natural appearance of the treated and coated material is enhanced. 40

11. In a process for coating a pervious material, first subjecting said material to mechanical treatment whereby the openings or interstices therein are reduced in size, applying to the face of said treated material a 45 coating material of the class comprising cellulose, celluloid compounds or mixtures, lacquers, varnishes or the like, and which will remain pliable in the coating, and subjecting the coated material to the action of steam or 50 moisture whereby the pliability and natural appearance of the treated and coated material is enhanced.

12. In a process for coating a pervious material, first applying pressure to said material whereby the openings or interstices therein are reduced in size, then applying to the face of said treated material a coating material of the class comprising cellulose, celluloid compounds or mixtures, lacquers, 55 varnishes or the like, and which will remain pliable in the coating and then subjecting the coated material to the action of steam or moisture whereby the pliability and natural 60 appearance of the treated and coated material 65 is enhanced.

In testimony whereof I have signed this specification.

NORMAN E. OLIVER.